# EUROPEAN PATENT SPECIFICATION

(11) **EP 1 439 877 B1**
(45) Date of publication and mention of the grant of the patent: **14.06.2006**
(21) Application number: 02777443.9
(22) Date of filing: 23.10.2002
(51) Int. Cl.: A61M 15/00, B65D 83/00, A61M 25/00, B65D 83/14

(54) **Method of producing a medicament dispenser**
Verfahren zur Herstellung eines Medikamentenspenders
Procédé de fabrication d'un distributeur de medicaments

(30) Priority: 23.10.2001 GB 0125380
(43) Date of publication of application: 28.07.2004
(73) Proprietor: GLAXO GROUP LIMITED, Greenford, Middlesex UB6 ONN (GB)
(72) Inventor: YASUDA, Hirotsugu, Colombia, MO 65203 (US); BONVOISIN, Cecile, Isabelle Laboratoire GlaxoSmith, B.P. 118, F-27091 Evreux Cedex 9 (FR); BRITTO, Ignatius, Loy Laboratoire GlaxoSmithKline, F-27091 Evreux Cedex 9 (FR); GREGER, Ralf, B-9700 Oudenaarde (BE); LAROCHE, Christophe Laboratoire GlaxoSmithKline, F-27091 Evreux Cedex 9 (FR); LO, Verna, Charlene GlaxoSmithKline, NC 27709 (US); PALMERS, Johan, B-7750 Amougies (BE); PEYRON, Isabelle, Denise GlaxoSmithKline, F-27091 Evreux Cedex 9 (FR); VANLANDEGHEM, Anthony, B-9700 Oudenaarde (BE)
(74) Representative: Rice, Jason Neale
(86) International application number: PCT/GB2002/004794
(87) International publication number: WO 2003/035154

(56) References cited:
- EP-A- 0 642 992
- WO-A-99/47195
- GB-A- 2 355 252
- US-A- 4 649 071
- US-A- 4 718 907
- US-A- 5 091 204
- US-A- 5 597 456
- US-A- 6 132 813
- US-A- 6 143 277

## Description

### Background of the Invention

Drugs for treating respiratory and nasal disorders are frequently administered in aerosol formulations through the mouth or nose. One widely used method for dispensing such aerosol drug formulations involves formulating the drug as a suspension or a solution in a liquefied gas propellant. The suspension/solution is stored in a sealed canister capable of withstanding the pressure required to maintain the propellant as a liquid. The suspension/solution is dispersed by activation of a dose-metering valve affixed to the canister.

A metering valve generally comprises a metering chamber, which is of a set volume and is designed to administer per actuation an accurate predetermined dose of medicament. As the suspension/solution is forced from the metering chamber through the valve stem by the high vapour pressure of the liquid propellant, the propellant rapidly vaporises leaving a fast moving cloud of very fine particles of the drug formulation. This cloud of particles is directed into the nose or mouth of the patient by a channelling device such as a cylinder or open-ended cone. Concurrently with the activation of the aerosol dose-metering valve, the patient inhales the drug particles into the lungs or nasal cavity. Systems of dispensing drugs in this way are known as "metered dose inhalers" (MDIs). See Peter Byron, Respiratory Drug Delivery, CRC Press, Boca Raton, FL (1990) for a general background on this form of therapy.

Patients often rely on medication delivered by MDls for rapid treatment of respiratory disorders, which are debilitating and in some cases even life threatening. Therefore, it is essential that the prescribed dose of aerosol medication delivered to the patient consistently meets the specifications claimed by the manufacturer and meets the requirements of regulatory authorities. That is, every dose in the can must be delivered within the same close tolerances.

A problem which can exist with drug delivery devices such as MDIs is deposition of medicament, or the solid component from a suspension of a particulate product in a liquid propellant, onto the internal surfaces of the device which occurs after a number of operation cycles and/or storage. A reduction in the efficacy of the device may occur. Deposition of the product also reduces the amount of active drug available to be dispensed to the patient and markedly reduces the uniformity of the dose dispensed during the lifetime of the device.

Drug deposition and adherence and dose uniformity may be greater with suspension formulations comprising hydrofluoroalkane propellants, for example, 1,1,1,2-tetrafluoroethane (HFA134a) and 1,1,1,2,3,3,3-n-heptafluoropropane (HFA227), which have been developed as ozone friendly replacements of chlorofluorocarbons such as P11, P114 and P12.

Some conventional devices rely on the dispenser being shaken, to agitate the liquid propellant and product mixture therein, in an attempt to re-suspend at least a portion of the deposited medicament. While in some cases this remedy can be effective within the body of the drug container itself, it may not be effective for particles deposited on the inner surface(s) of other MDI components such as the metering valve.

Canadian patent application 2130867 describes a metered dose inhaler containing an aerosol formulation in which the internal walls of the metal canister are coated with a cross-linked plastics coating. Polytetrafluoroethylene (PTFE) and perfluoroethylenepropylene (FEP) are specifically mentioned as suitable coating materials.

UK patent application GB-A-2,328,932 discloses the use of a liner of a material such as fluoropolymer, ceramic or glass to line a portion of the wall of the metering chamber in a metering valve of an MDI. Although this alleviates the problem of deposition in these types of dispensers, it does require the re-design or modification of mouldings and mould tools for producing the valve members to allow for insertion of the liner.

WO-A-99/47195 discloses a method according to the pre-characterising part of claim 1 thereof.

US-A-5597456 discloses use of a plasma treatment to form an anti-thrombotic material.

### Summary of the Invention

It is therefore an aim of the present invention to provide a highly fluorinated, reproducible coating which prevents or inhibits adhesion of drug particles to the internal surfaces of the canister and/or valve components of a medicament dispenser, for example an MDI.

It is a further aim of the present invention to provide a coating with reduces moisture ingress into a medicament formulation, for example a pharmaceutical aerosol formulation, reduces drug absorption into the internal surface, especially when of rubber, and reduces extractables leached out from the internal surface, especially when of plastics and rubber components.

### Detailed Description of the Invention

Accordingly, the invention provides a method according to claim 1 thereof.

Suitably, the fluorinated coating has a fluorine/carbon atomic ratio of greater than 10% about 1.0 and preferably greater than about 1.2, when measured by Electronic Spectroscopy for Chemical Analysis (ESCA), also referred to as X-ray photo Spectroscopy (XPS).

Suitably, the fluorinated coating comprises greater than about 10% CF₂ units and greater than about 10% CF₂CF units, the CF₂ and CF₂CF units being present either as part of a Teflon moiety or as a separate moiety. The percentage of CF₂ and CF₂CF units may be measured using ESCA.

Suitably, the surface energy of the coating gives a contact angle of greater than about 80 degrees, preferably greater than about 90 degrees. The term "contact angle" is the angle between a liquid water droplet and the coated surface of the canister/valve at the liquid/solid interface as measured in ambient conditions, i.e. at a temperature of 20°C (± 5°C) and a relative humidity of 50% (± 20%). The contact angle may be measured on a coating deposited on a flat polybutylene terephthalate (PBT) substrate surface in accordance with the invention.

The thickness of the fluorinated coating is in the range of about 1 to about 200nm, suitably about 10 to 100nm, and preferably about 20 to 80nm.

In one embodiment, one or more internal surfaces of the canister comprise the fluorinated coating produced by the method of the invention. In addition, or alternatively, one or more produced by the method internal surfaces of the valve may comprise the fluorinated coating produced by the method the invention.

Any parts of the canister or valve which contact the pharmaceutical aerosol suspension may be coated with the fluorinated coating produced by the method of the invention. The fluorinated coating reduces or eliminates the tendency for medicament particles to adhere to such component surfaces. Where the valve part is a movable part (e.g. the valve stem) the coating also reduces the friction between that part and an adjacent part of the valve (e.g. the stem seal).

As known by a person skilled in the art, the drug-dispensing valve suitably comprises a number of components or parts. All of these may, independently of the other components, be coated with a fluorinated coating as hereinbefore defined. Component parts of the valve which may be coated include, but are not limited to, the metering chamber, valve stem, the upper and lower stem seals, neck gasket, spring, body, and the ring.

In one aspect herein, the valve stem is provided with the coating produced by the method of the invention to reduce its frictional contact properties, and the need for any further stem lubricant such as silicone oil is reduced or eliminated. Reducing frictional-contact can be particularly advantageous where the valve is employed in a dispenser for both suspension and solution medicament formulations.

In a further aspect, one or more internal surfaces of the metering chamber are provided with a fluorinated coating produced by the method according to the present invention.

In a still further aspect, one or more component parts selected from the group consisting of the upper and lower stem seals, neck gasket, spring, body, and ring are provided with a fluorinated coating produced by the method according to the present invention.

The dispenser may be incorporated as part of a "metered dose inhaler" ("MDI" for short) for dispensing a medicament in a fluid propellant under pressure. The term "MDI" means a unit comprising a canister, a ferrule covering the mouth of the canister, a drug metering valve situated in the ferrule, a metering chamber and a suitable channelling device into which the canister is fitted. The relation of the parts of a typical MDI is illustrated in US Patent 5,261,538.

Optionally, moisture-absorbing means is further comprised within the dispenser or metered dose inhaler as a component thereof. Examples of moisture absorbing means suitable for use are disclosed in WO-A-02/30499.

The coating applied to one or more internal surfaces of the canister and/or valve is prepared from a plasma generated substantially from a fluorinated monomer selected from the group consisting of CH₂FCF₃. Alternatively, the fluorinated monomer selected from the group consisting of CH₂FCF₃ may be co-polymerised with one or more additional non-fluorinated monomers. Suitable copolymers compose from 0.5 to 99.5% by weight, preferably from 0.7 to 85% by weight, of fluorinated monomer, In general the preference is to use a non-fluorinated monomer that forms the basic building block (monomer) of the substrate polymer or elastomer to be coated. For example, if polybutylene terephthalate (PBT) is the substrate to be coated, the monomer used in producing PBT, dimethyl terephthalate, can be used in conjunction with the fluorinated monomer. Similarly, if the substrate is acetal, then CH₂O can be used in general, irrespective of the substrate material, when fluorinated coatings are produced using a plasma process, it is desirable to use basic hydrocarbon monomers, including, but not limited to, CH₄, C₂H₆, C₂H₄, N₂, O₂, H₂, C₃COO(C₆H₆)COOCH₃, HO(CH₂)₂OH, C₃H₃N and C₄H₆ in conjunction with the fluorinated monomer.

The ratio of the gas flow rate of the fluorinated monomer to the non-fluorinated monomer can be continuously varied during the course of the plasma coating process. In general, in order to obtain superior adhesion, this ratio can be low or the monomer gas can be rich in the non-fluorinated species at the start of the process. This ratio can be continuously increased and towards the end of the process it is preferable to use only the fluorinated monomer in order to obtain a fluorine rich surface in the top layers of the coating.

The fluorinated coating is prepared using a plasma polymerisation process; suitably a RF plasma polymerisation process operating at a frequency of 2MHz to 200MHz; suitably 13.56MHz, 27.12MHz and 40.68MHz; and preferably 13.56MHz. The coating process typically occurs under vacuum. The components to be coated are placed inside a rotating chamber, the chamber subsequently being evacuated. The fluorinated monomer (and optionally additional monomeric material) is introduced into the chamber, suitably at ambient temperature, and at a controlled and predetermined flow rate. The monomer gas(es) is ignited and dissociates into plasma within the chamber. The energy in the chamber is maintained for a given time at a chosen power setting. During plasma polymerisation electrode temperatures can typically increase from about 20°C to about 100°C. A cooling system of the electrode is used to minimise the temperature increase. At the end of the treatment the plasma is extinguished, the chamber flushed with air or argon and the coated products retrieved. During the polymerisation process, a thin layer of plasma polymer will be bonded to the canister and/or valve component. The polymerisation process time may only be minutes, for instance 30 minutes or less, or as long as several hours, depending on the operating conditions etc., as will be understood by the skilled reader in the art.

Accordingly, application of the fluorinated coating may be by a process comprising the steps of (i) placing the canister and/or valve component to be coated in a chamber, (ii) evacuating the chamber, (iii) feeding CH₂FCF₃ gas into the chamber, (iv) applying sufficient power to generate a plasma, (v) igniting the plasma, (vi) extinguishing any unreacted plasma, and (vii) flushing the chamber.

One or more additional non-fluorinated monomers may also be fed into the chamber. Suitably, the ratio of fluorinated to non-fluorinated gas flow rate is continuously varied during the process. More suitably, the ratio of fluorinated to non-fluorinated gas flow rate is increased during the process. Preferably, the monomer gas is pure non-fluorinated monomer at the start of the process and pure fluorinated monomer at the end of the process.

The effectiveness of the fluorinated coating may depend on the operating conditions of the plasma reactor. The operating parameters, which can be varied, include: power (W), gas pressure (mTorr), gas flow (cc/min), tumbler speed (rpm), temperature (°C) and the number of components in the chamber.

Suitably, the reactor operates at a power of between 50W and 450W, suitably 75W and 300W and preferably about 200W.

Suitably, the reactor operates at a gas pressure of loss than or equal to about 70mTorr.

Suitably, the reactor operates at a gas flow of between 50cc/min and 200cc/min; suitably between 75cc/min and 100cc/min.

Suitably, the reactor operates at a tumbler speed of between 1 and 15rpm, suitably at about 3rpm or 8rpm.

Suitably, the temperature of the electrode increases from 20°C to 100°C.

The positioning of the components within the reactor may affect the effectiveness of the coating. The components to be coated should be positioned within the primary plasma in the reactor (inside the glow of the plasma). In order to obtain a uniform coating on all the components, the components should be evenly distributed in the reactor and then rotated.

Suitably, to improve adhesion of the fluorinated coating to the internal surfaces, the surfaces to be coated may be subjected to a pre-treatment procedure to remove any surface contamination and/or to activate the surface. Accordingly, the internal surface(s) of the canister and/or valve are subjected to a pre-treatment step to remove surface contamination and/or to activate the surface prior to providing a fluorinated coating as hereinbefore described. The pre-treatment step may be carried out by for example plasma treatment of the components with an etching gas such as oxygen or a neutral gas such as argon. Preferably, the gas is argon to avoid damage to the substrate. In the process, radicals react with the plastic or metal substrate; for example the component is exposed to a tow pressure argon plasma environment generating polar groups on the component's surface. Such polar groups are more conducive to bonding with the fluorine-containing plasma coating to be applied.

The pre-treatment step, for example with argon, could be carried out under a range of conditions and duration. However, the following conditions provide a satisfactory pre-treatment for a PBT substrate: run time 5 minutes; power 300W; gas pressure 80mTorr, gas flow 150cc/min; tumbler speed 3rpm or 8rpm. It should be noted, however, that the invention is not limited to these conditions and that any set of conditions used for a pre-treatment step is within the scope of the invention. The pre-treatment process is dependent on the material to be treated.

The metered dose inhalers may be prepared by methods known in the art, for example as disclosed in Byron *supra* and US patent 5,345,980.

Suitably, the entire valve or one or more of the valve components are made of a non-metal material. Suitable non-metals for use in the valve include pharmacologically resilient polymers such as acetal, polyamide (e.g. Nylon®), polycarbonate, polyester (e.g. polybutylene terephthalate (PBT)), fluorocarbon polymer (e.g. Teflon®) or a combination of these materials. Additionally, seals and "O" rings of various materials (e.g., nitrile rubbers, polyurethane, acetyl resin, fluorocarbon polymers), or other elastomeric materials, for example EPDM, and thermoplastic elastomer or chloroprene, are employed in and around the valve. Alternatively, the valve is made of metal, for example stainless steel, aluminium, copper, tin plate and any alloys thereof.

The valve can have any suitable configuration. Metal and non-metal parts can be combined to optimise the performance of the valve.

Conventionally, the canisters and caps for use in MDls are made of aluminium or an alloy of aluminium although other metals not affected by the drug formulation, such as stainless steel, an alloy of copper, or tin plate, may be used. An MDI canister may also be fabricated from glass or plastics. Preferably, however, the MDI canisters and caps employed in the present invention are made of aluminium or an alloy thereof.

The canister, when in use, is a pressurised container comprising a vial (preferably metal, more preferably aluminium) having a metering valve disposed therein. Since the canister is preferably part of an MDI, the metering valve design is typically a function of providing a predetermined dosage or amount of the drug contained within the pressurised container to a user.

The valve typically comprises a valve body having an inlet port through which the pharmaceutical aerosol formulation may enter said valve body, an outlet port through which the pharmaceutical aerosol may exit the valve body and an open/close mechanism by means of which flow through said outlet port is controllable.

The valve may be a slide valve wherein the open/close mechanism comprises a sealing ring and receivable by the sealing ring a valve stem having a dispensing passage, the valve stem being slidably movable within the ring from a valve-closed to a valve-open position in which the interior of the valve body is in communication with the exterior of the valve body via the dispensing passage.

The metering volumes are typically from 25 to 100 µl, such as 50 µl or 63 µl. Suitably, the valve body defines a metering chamber for metering an amount of medicament formulation and an open/close mechanism by means of which the flow through the inlet port to the metering chamber is controllable. Preferably, the valve body has a sampling chamber in communication with the metering chamber via a second inlet port, said inlet port being controllable by means of an open/close mechanism thereby regulating the flow of medicament formulation into the metering chamber.

The valve may be a metering valve in which the valve body has a metering chamber, a sampling chamber and therebetween a second sealing ring within which the stem is slidably movable, the valve stem having a transfer passage such that in the valve-closed position the dispensing passage is isolated from the metering chamber and the metering chamber is in communication with the sampling chamber via the transfer passage, and in the valve-open position the dispensing passage is in communication with the metering chamber and the transfer passage is isolated from the metering chamber.

The valve may also comprise a 'free flow aerosol valve' having a chamber and a valve stem extending into the chamber and movable relative to the chamber between dispensing and non-dispensing positions. The valve stem has a configuration and the chamber has an internal configuration such that a metered volume is defined therebetween and such that during movement between non-dispensing and dispensing positions the valve stem sequentially: (i) allows free flow of aerosol formulation into the chamber, (ii) defines a closed metered volume for pressurised aerosol formulation between the external surface of the valve stem and internal surface of the chamber, and (iii) moves with the closed metered volume within the chamber without decreasing the volume of the closed metered volume until the metered volume communicates with an outlet passage thereby allowing dispensing of the metered volume of pressurised aerosol formulation. A valve of this type is described in U.S. Patent No. 5,772,085.

The valve may also have a structure and action similar to those aerosol valves described in European Patent Application No. EP-A-870,699 and PCT Patent Application No. WO99/36334.

The sealing ring and/or gasket may be formed by cutting a ring from a sheet of suitable material. Alternatively, the sealing ring and/or gasket may be formed by a moulding process such as an injection moulding, a compression moulding or a transfer moulding process.

Typically, the sealing ring and/or second sealing ring and/or gasket comprise an elastomeric material. The ring is typically resiliently deformable.

The elastomeric material may either comprise a thermoplastic elastomer (TPE) or a thermoset elastomer, which may optionally be cross-linked. The sealing ring and/or gasket may also comprise a thermoplastic elastomer blend or alloy in which an elastomeric material is dispersed in a thermoplastic matrix. The elastomers may optionally additionally contain conventional polymer additives. Such additives include but are not limited to processing aids, colorants, tackifiers, lubricants, silica, talc, or processing oils such as mineral oil in suitable amounts.

Suitable thermoset rubbers include butyl rubbers, chloro-butyl rubbers, bromo-butyl rubbers, nitrile rubbers, silicone rubbers, fluorosilicone rubbers, fluorocarbon rubbers, polysulphide rubbers, polypropylene oxide rubbers, isoprene rubbers, isoprene-isobutene rubbers, isobutylene rubbers or neoprene (polychloroprene) rubbers.

Suitable thermoplastic elastomers comprise a copolymer of about 80 to about 95 mole percent ethylene and a total of about 5 to about 20 mole percent of one or more comonomers selected from the group consisting of 1-butene, 1-hexene, and 1-octene as known in the art. Two or more such copolymers may be blended together to form a thermoplastic polymer blend.

Another suitable class of thermoplastic elastomers are the styrene-ethylene/butylene-styrene block copolymers. These copolymers may additionally comprise a polyolefin (e.g. polypropylene) and a siloxane.

Thermoplastic elastomeric material may also be selected from one or more of the following: polyester rubbers, polyurethane rubbers, ethylene vinyl acetate rubber, styrene butadiene rubber, copolyether ester TPE, olefinic TPE, polyester amide TPE and polyether amide TPE.

Other suitable elastomers include ethylene propylene diene rubber (EPDM). The EPDM may be present on its own or present as part of a thermoplastic elastomer blend or alloy, e.g. in the form of particles substantially uniformly dispersed in a continuous thermoplastic matrix (e.g. polypropylene or polyethylene). Commercially available thermoplastic elastomer blend and alloys include the SANTOPRENE^{™} elastomers. Other suitable thermoplastic elastomer blends include butyl-polyethylene (e.g. in a ratio ranging between about 2:3 and about 3:2) and butyl-polypropylene.

Typically, the sealing ring and/or the second sealing ring and/or gasket additionally comprises lubricant material. Suitably, the sealing ring and/or the second sealing ring and/or gasket comprises up to 30% by weight, preferably from 5 to 20% by weight, of lubricant material.

In addition, the stem may also comprise lubricant material. Suitably, the valve stem comprises up to 30%, preferably from 5 to 20% lubricant material by weight.

The term 'lubricant' herein means any material that reduces friction between the valve stem and seal. Suitable lubricants include silicone oil or a fluorocarbon polymer such as polytetrafluoroethane. (PTFE) or tluoroethylene propylene (FEP).

Lubricant can be applied to the stem, stem gaskets or ferrule by any suitable process including coating and impregnation, such as by injection or by adding a reservoir of lubricant, which provides a constant supply of lubricant throughout the life of the product.

In medical use the canisters contain a pharmaceutical aerosol formulation comprising particles of a medicament and a hydrofluoroalkane propellant of 1,1,1,2-tetrafluoroethane (CF₃GH₂F).

The pharmaceutical formulations for use in the canisters contain no components that provoke the degradation of stratospheric ozone. In particular the formulations are substantially free of chlorofluorocarbons such as CCl₃F, CCl₂F₂ and CF₃CCl₃.

The propellant may additionally contain a volatile adjuvant such as a saturated hydrocarbon for example propane, n-butahe, isobutane, pentane and isopentane or a dialkyl ether for example dimethyl ether. In general up to 50% w/w of the propellant may comprise a volatile hydrocarbon, for example 1 to 30% w/w. However, formulations which are free or substantially free of volatile adjuvants are preferred, In certain cases, it may be desirable to include appropriate amounts of water, which can be advantageous in modifying the dielectric properties of the propellant.

A polar co-solvent such as C₂₋₆ aliphatic alcohols and polyols e.g. ethanol, isopropanol and propylene glycol, preferably ethanol, may be included in the drug formulation in the desired amount to improve the dispersion of the formulation, either as the only excipient or in addition to other excipients such as surfactants. Suitably, the drug formulation may contain 0.01 to 30% w/w based on the propellant of a polar co-solvent e.g. ethanol, preferably 0.1 to 20% w/w e.g. about 0.1 to 15% w/w. In aspects herein, the solvent is added in sufficient quantities to solubilise a part of, or all of, the medicament component, such formulations being commonly referred to as solution formulations.

A surfactant may also be employed in the aerosol formulation. Examples of conventional surfactants are disclosed in EP-A-372,777. The amount of surfactant employed is desirable in the range 0.0001% to 50% weight to weight ratio relative to the medicament, in particular, 0.05 to 5% weight to weight ratio.

The final aerosol formulation desirably contains 0.005-10% w/w, preferably 0.005 to 5% w/w, especially 0.01 to 1.0% w/w, of medicament relative to the total weight of the formulation.

Medicaments, which may be administered in the aerosol formulations, include any drug useful in inhalation therapy. The dispenser is suitable for dispensing medicament for the treatment of respiratory disorders such as disorders of the lungs, and bronchial tracts including asthma and chronic obstructive pulmonary disorder (COPD). The dispenser is suitable for dispensing medicament for the treatment of a condition requiring treatment by the systemic circulation of medicament, for example migraine, diabetes, pain relief e.g. inhaled morphine.

Accordingly, the dispenser or MDI may be used for the treatment of a respiratory disorder, such as asthma and COPD.

In addition the dispenser or MDI may be used for the treatment of a condition requiring the systemic circulation of a medicament, such as, for example, migraine, diabetes, chronic pain.

Appropriate medicaments may thus be selected from, for example, analgesics, e.g., codeine, dihydromorphine, ergotamine, fentanyl or morphine; anginal preparations, e.g., diltiazem; antiallergics, e.g., cromoglycate (e.g. as the sodium salt), ketotifen or nedocromil (e.g. as the sodium salt); antiinfectives e.g., cephalosporins, penicillins, streptomycin, sulphonamides, tetracyclines and pentamidine; antihistamines, e.g., methapyrilene; anti-inflammatories, e.g., beclbmethasone (e.g. as the dipropionate ester), fluticasone (e.g. as the propionate or furoate ester), flunisolide, budesonide, rofleponide, mometasone (e.g. as the furoate ester), ciclesonide, triamcinolone (e.g. as the acetonide) or 6α, 9α-difluoro-11β-hydroxy-16α-methyl-3-oxo-17α-proprionyloxy-androsta-1,4-diene-17β-carbothioic acid S-(2-oxo-tetrahydro-furan-3-yl) ester; antitussives, e.g., noscapine; bronchodilators, e.g., albuterol (e.g. as free base or sulphate), salmeterol (e.g. as xinafoate), ephedrine, adrenaline, fenoterol (e.g. as hydrobromide), formoterol (e.g. as fumarate), isoprenaline, metaproterenol, phenylephrine, phenylpropanolamine, pirbuterol (e.g. as acetate), reproterol (e.g. as hydrochloride), rimiterol, terbutaline (e.g. as sulphate), isoetharine, tulobuterol or 4-hydroxy-7-[2-[[2-[[3-(2-phenylethoxy)propyl]sulfonyl] ethyl]amino]ethyl-2(3H)-benzothiazolone; adenosine 2a agonists; e.g. 2R,3R,4S,5R)-2-[6-Amino-2-(1S-hydroxymethyl-2-phenylethylamino)-purin-9-yl]-5-(2-ethyl-2H-tetrazol-5-yl)-tetrahydro-furan-3,4-diol (e.g. as maleate); α₄ integrin inhibitors e.g. (2S)-3-[4-({[4-(aminocarbonyl)-1-pipendinyl]carbonyl}oxy)phenyl]-2-[((2S)-4-methyl-2-{[2-(2-methylphenoxy) acetyl]amino}pentanoyl)amino] propanoic acid (e.g. as free acid or potassium salt), diuretics, e.g., amiloride; anticholinergics, e.g., ipratropium (e.g. as bromide), tiotropium, atropine or oxitropium; hormones, e.g., cortisone, hydrocortisone or prednisolone; xanthines, e.g., aminophylline, choline theophyllinate, lysine theophyllinate or theophylline; therapeutic proteins and peptides, e.g., insulin or glucagon; vaccines, diagnostics, and gene therapies. It will be clear to a person skilled in the art that, where appropriate, the medicaments may be used the form of salts, (e.g., as alkali metal or amine salts or as acid addition salts) or as esters (e.g., lower alkyl esters) or as solvates (e.g. hydrates) to optimise the activity and/or stability of the medicament.

Preferred medicaments are selected from albuterol, salmeterol, fluticasone propionate and beclomethasone dipropionate and salts or solvates thereof, e.g., the sulphate of albuterol and the xinafoate of salmeterol.

Medicaments can also be delivered in combinations. Preferred formulations containing combinations of active ingredients contain salbutamol (e.g., as the free base or the sulphate salt) or salmeterol (e.g., as the xinafoate salt) or formoterol (e.g., as the fumarate salt) in combination with an anti-inflammatory steroid such as a beclomethasone ester (e.g., the dipropionate) or a fluticasone ester (e.g., the propionate) or budesonide. A particularly preferred combination is a combination of fluticasone propionate and salmeterol, or a salt thereof (particularly the xinafoate salt). A further combination of particular interest is budesonide and formoterol (e.g. as the fumarate salt).

Conventional bulk manufacturing methods and machinery well known to those skilled in the art of pharmaceutical aerosol manufacture may be employed for the preparation of large scale batches for the commercial production of filled canisters. Thus, for example, in one bulk manufacturing method a metering valve is crimped onto an aluminium can to form an empty canister. The particulate medicament is added to a charge vessel and liquefied propellant is pressure filled through the charge vessel into a manufacturing vessel. The drug suspension is mixed before re-circulation to a filling machine and an aliquot of the drug suspension is then filled through the metering valve into the canister. Typically, in batches prepared for pharmaceutical use, each filled canister is check-weighed, coded with a batch number and packed into a tray for storage before release testing.

Each filled canister is conveniently fitted into a suitable channelling device prior to use to form a metered dose inhaler for administration of the medicament into the lungs or nasal cavity of a patient. Suitable channelling devices comprise for example a valve actuator and a cylindrical or cone-like passage through which medicament may be delivered from the filled canister via the metering valve to the nose or mouth of a patient e.g. a mouthpiece actuator. Metered dose inhalers are designed to deliver a fixed unit dosage of medicament per actuation or "puff", for example in the range of 2 to 5000 microgram medicament per puff.

Administration of medicament may be indicated for the treatment of mild, moderate or severe acute or chronic symptoms or for prophylactic treatment. It will be appreciated that the precise dose administered will depend on the age and condition of the patient, the particular particulate medicament used and the frequency of administration and will ultimately be at the discretion of the attendant physician. When combinations of medicaments are employed the dose of each component of the combination will in general be that employed for each component when used alone. Typically, administration may be one or more times, for example from 1 to 8 times per day, giving for example 1,2,3 or 4 puffs each time. Each valve actuation, for example, may deliver 5µg, 50µg, 100µg, 200µg or 250µg of a medicament. Typically, each filled canister for use in a metered dose inhaler contains 60, 100, 120 or 200 metered doses or puffs of medicament; the dosage of each medicament is either known or readily ascertainable by those skilled in the art.

For the avoidance of doubt, the use herein of the term "about" in reference to the value(s) of certain parameters is meant to include the exact value of that parameter, e.g. a reference to the relative amount of a material being "about Xg by weight" encompasses the relative amount being exactly Xg by weight.

## Claims

1. A method of producing a dispenser for dispensing a medicament comprising a canister housing particles of the medicament in a fluid propellant of 1,1,1,2-tetrafluoroethane and a drug-dispensing valve, said method including the step of applying to one or more of the internal surfaces of the canister and/or valve a fluorinated coating by plasma polymerisation, **characterised in that** the plasma polymerisation is of CH₂FCF₃.

2. A method according to claim 1, wherein the fluorinated coating has a fluorine/carbon atomic ratio of greater than about 1.0.

3. A method according to claim 2, wherein the fluorine/carbon atomic ratio is greater than about 1.2.

4. A method according to any preceding claim, wherein the fluorinated coating comprises greater than about 10% CF₂ units.

5. A method according to any preceding claim, wherein the fluorinated coating comprises greater than about 10%CF₂CF units.

6. A method according to any preceding claim, wherein the fluorinated coating gives a contact angle of greater than about 80°.

7. A method according to claim 6, wherein the fluorinated coating gives a contact angle of greater than about 90°.

8. A method according to any preceding claim, wherein the fluorinated coating has a thickness in the range of about 1 to 200nm.

9. A method according to claim 8, wherein the thickness is in the range of about 10 to 100nm.

10. A method according to any preceding claim, wherein the fluorinated coating is provided on one or more internal surfaces of the canister.

11. A method according to any one of claims 1 to 10, wherein the fluorinated coating is provided on one or more internal surfaces of the valve.

12. A method according to claim 11, wherein the fluorinated coating is provided on one or more internal surfaces of a metering chamber of the valve.

13. A method according to claim 12, wherein the fluorinated coating is provided on a valve stem of the valve.

14. A method according to claim 11, wherein the fluorinated coating is provided on one or more valve component parts selected from the group consisting of an upper stem seal, a lower stem seal, a neck gasket, a spring, a body and a ring.

15. A method according to any preceding claim, wherein the fluorinated coating is prepared from the plasma co-polymerisation of CH₂FCF₃ and one or more additional non-fluorinated monomers.

16. A method according to claim 15, wherein the one or more additional non-fluorinated monomers are selected from the group consisting of CH₄, C₂H₆, C₂H₄, N₂, O₂, H₂, C₃COO(C₆H₆)COOCH₃, HO(CH₂)₂OH, C₃H₃N and C₄H₆.

17. A method according to any preceding claim in which the the fluorinated coating is applied by a process comprising the steps of (i) placing the component to be coated in a chamber, (ii) evacuating the chamber, (iii) feeding CH₂FCF₃ gas into the chamber, (iv) applying sufficient power to generate a plasma, (v) igniting the plasma, (vi) extinguishing any unreacted plasma, and (vii) flushing the chamber.

18. A method according to claim 17, wherein one or more additional non-fluorinated monomer gases are fed into the chamber.

19. A method according to claim 18, wherein the ratio of the CH₂FCF₃ gas flow rate to the non-fluorinated gas flow rate is continuously varied during the process.

20. A method according to any one of claims 18 to 19, wherein the ratio of the CH₂FCF₃ gas flow rate to the non-fluorinated gas flow rate is increased during the process.

21. A method according to any one of claims 18 to 20, wherein the gas is pure non-fluorinated monomer at the start of the process and pure CH₂FCF₃ gas at the end of the process.

22. A method according to any one of claims 17 to 21, wherein the process is carried out at a power from 50W to 450W.

23. A method according to any one of claims 17 to 22, wherein the process is carried out at a gas pressure of less than or equal to 70m Torr.

24. A method according to any one of claims 17 to 23, wherein the process is carried out at a gas flow rate from 50cc/min to 200cc/min.

25. A method according to any one of claims 17 to 24, wherein the process is carried out at a tumbler speed from 1 to 15rpm.

26. A method according to any one of claims 17 to 25, wherein the process is carried out at a temperature from 20°C to 100°C.

27. A method according to any one of claims 17 to 26, wherein the plasma polymerisation process is carried out at a radio frequency in the range of 2MHz to 200MHz.

28. A method according to claim 27, wherein the radio frequency is approximately 13.56MHz.

29. A method according to any one of claims 17 to 28 in which the plasma is maintained for a duration of 30 minutes, or substantially 30 minutes.

30. A method according to any one of claims 17 to 29, wherein said process comprises a pre-treatment step to remove surface contamination and/or activate the surface.

31. A method according to claim 30, wherein said pre-treatment step comprises plasma treatment of the components with oxygen or argon.

## Patentansprüche

1. Verfahren zur Herstellung einer Ausgabevorrichtung zum Ausgeben eines Medikaments, die einen Kanister, der Teilchen des Medikaments in einem fluiden Treibmittel aus 1,1,1,2-Tetrafluorethan aufnimmt, und ein Wirkstoff-Ausgabeventil umfasst, wobei das Verfahren den Schritt des Auftragens einer fluorierten Beschichtung auf eine oder mehrere der Innenoberflächen des Kanisters und/oder des Ventils durch Plasmapolymerisation einschliesst, **dadurch gekennzeichnet, dass** die Plasmapolymerisation von CH₂FCF₃ ist.

2. Verfahren gemäss Anspruch 1, worin die fluorierte Beschichtung ein Fluor/Kohlenstoff-Atomverhältnis von mehr als 1,0 aufweist.

3. Verfahren gemäss Anspruch 2, worin das Fluor/Kohlenstoff-Atomverhältnis grösser als ca. 1,2 ist.

4. Verfahren gemäss jedem vorhergehenden Anspruch, worin die fluorierte Beschichtung mehr als ca. 10 % CF₂-Einheiten umfasst.

5. Verfahren gemäss jedem vorhergehenden Anspruch, worin die fluorierte Beschichtung mehr als ca. 10 % CF₂CF-Einheiten umfasst.

6. Verfahren gemäss jedem vorhergehenden Anspruch, worin die fluorierte Beschichtung einen Kontaktwinkel von mehr als ca. 80° ergibt.

7. Verfahren gemäss Anspruch 6, worin die fluorierte Beschichtung einen Kontaktwinkel von mehr als ca. 90° ergibt.

8. Verfahren gemäss jedem vorhergehenden Anspruch, worin die fluorierte Beschichtung eine Dicke im Bereich von ca. 1 bis 200 nm hat.

9. Verfahren gemäss Anspruch 8, worin die Dicke im Bereich von ca. 10 bis 100 nm ist.

10. Verfahren gemäss jedem vorhergehenden Anspruch, worin die fluorierte Beschichtung auf einer oder mehreren Innenoberflächen des Kanisters vorgesehen wird.

11. Verfahren gemäss einem der Ansprüche 1 bis 10, worin die fluorierte Beschichtung auf einer oder mehreren Innenoberflächen des Ventils vorgesehen wird.

12. Verfahren gemäss Anspruch 11, worin die fluorierte Beschichtung auf einer oder mehreren Innenoberflächen einer Dosierkammer des Ventils vorgesehen wird.

13. Verfahren gemäss Anspruch 12, worin die fluorierte Beschichtung auf einem Ventilschaft des Ventils vorgesehen wird.

14. Verfahren gemäss Anspruch 11, worin die fluorierte Beschichtung auf einem oder mehreren Ventilkomponententeilen vorgesehen wird, die aus der Gruppe ausgewählt sind, die aus einer oberen Schaftdichtung, einer unteren Schaftdichtung, einer Halsdichtung, einer Feder, einem Körper und einem Ring besteht.

15. Verfahren gemäss jedem vorhergehenden Anspruch, worin die fluorierte Beschichtung aus der Plasma-Copolymerisation von CH₂FCF₃ und einem oder mehreren zusätzlichen nicht-fluorierten Monomeren hergestellt wird.

16. Verfahren gemäss Anspruch 15, worin das eine oder die mehreren zusätzlichen nicht-fluorierten Monomere aus der Gruppe ausgewählt sind, die aus CH₄, C₂H₆, C₂H₄, N₂, O₂, H₂, C₃COO(C₆H₆)COOCH₃, HO(CH₂)₂OH, C₃H₃N und C₄H₆ besteht.

17. Verfahren gemäss jedem vorhergehenden Anspruch, worin die fluorierte Beschichtung durch einen Prozess aufgetragen wird, der die folgenden Schritte umfasst: (i) Stellen der zu beschichtenden Komponente in eine Kammer, (ii) Evakuieren der Kammer, (iii) Zuführen von CH₂FCF₃-Gas in die Kammer, (iv) Anlegen von ausreichender Leistung, um ein Plasma zu erzeugen, (v) Zünden des Plasmas, (vi) Löschen von etwaigem nicht reagiertem Plasma und (vii) Spülen der Kammer.

18. Verfahren gemäss Anspruch 17, worin ein oder mehrere zusätzliche nicht-fluorierte Monomergase der Kammer zugeführt werden.

19. Verfahren gemäss Anspruch 18, worin das Verhältnis der Fliessgeschwindigkeit des CH₂FCF₃-Gases zur Fliessgeschwindigkeit des nicht-fluorierten Gases während des Prozesses kontinuierlich variiert wird.

20. Verfahren gemäss einem der Ansprüche 18 bis 19, worin das Verhältnis der Fliessgeschwindigkeit des CH₂FCF₃₋Gases zur Fliessgeschwindigkeit des nicht-fluorierten Gases während des Prozesses erhöht wird.

21. Verfahren gemäss einem der Ansprüche 18 bis 20, worin das Gas reines nicht-fluoriertes Monomer zu Beginn des Prozesses und reines CH₂FCF₃-Gas am Ende des Prozesses ist.

22. Verfahren gemäss einem der Ansprüche 17 bis 21, worin der Prozess mit einer Leistung von 50 bis 450 W durchgeführt wird.

23. Verfahren gemäss einem der Ansprüche 17 bis 22, worin der Prozess bei einem Gasdruck von 70 mTorr oder weniger durchgeführt wird.

24. Verfahren gemäss einem der Ansprüche 17 bis 23, worin der Prozess bei einer Gasfliessgeschwindigkeit von 50 bis 200 cm³/min durchgeführt wird.

25. Verfahren gemäss einem der Ansprüche 17 bis 24, worin der Prozess bei einer Tumbler-Geschwindigkeit von 1 bis 50 U/min durchgeführt wird.

26. Verfahren gemäss einem der Ansprüche 17 bis 25, worin der Prozess bei einer Temperatur von 20 bis 100°C durchgeführt wird.

27. Verfahren gemäss einem der Ansprüche 17 bis 26, worin der Plasmapolymerisationsprozess bei einer Hochfrequenz im Bereich von 2 bis 200 MHz durchgeführt wird.

28. Verfahren gemäss Anspruch 27, worin die Hochfrequenz ca. 13,56 MHz ist.

29. Verfahren gemäss einem der Ansprüche 17 bis 28, worin das Plasma für eine Dauer von 30 Minuten oder im wesentlichen 30 Minuten aufrechterhalten wird.

30. Verfahren gemäss einem der Ansprüche 17 bis 29, worin der Prozess einen Vorbehandlungsschritt zur Entfernung von Oberflächenverunreinigung und/oder zur Aktivierung der Oberfläche umfasst.

31. Verfahren gemäss Anspruch 30, worin der Vorbehandlungsschritt die Plasmabehandlung der Komponenten mit Sauerstoff oder Argon umfasst.

## Revendications

1. Procédé de production d'un appareil distributeur pour distribuer un médicament comprenant une boîte logeant des particules du médicament dans un propulseur fluide de 1,1,1,2-tétrafluoroéthane et une vanne de distribution du médicament, ledit procédé comprenant l'étape consistant à appliquer à une ou plusieurs des surfaces internes de la boîte et/ou de la vanne un revêtement fluoré par polymérisation plasma, **caractérisé en ce que** la polymérisation plasma est une polymérisation de CH₂FCF₃.

2. Procédé selon la revendication 1, dans lequel le revêtement fluoré a un rapport atomique du fluor au carbone supérieur à environ 1,0.

3. Procédé selon la revendication 2, dans lequel le rapport atomique du fluor au carbone est supérieur à environ 1,2.

4. Procédé selon l'une quelconque des revendications précédentes, dans lequel le revêtement fluoré comprend plus d'environ 10% d'unités de CF₂.

5. Procédé selon l'une quelconque des revendications précédentes, dans lequel le revêtement fluoré comprend plus d'environ 10 % d'unités de CF₂CF.

6. Procédé selon l'une quelconque des revendications précédentes, dans lequel le revêtement fluoré donne un angle de contact supérieur à environ 80°.

7. Procédé selon la revendication 6, dans lequel le revêtement fluoré donne un angle de contact de plus d'environ 90°.

8. Procédé selon l'une quelconque des revendications précédentes, dans lequel le revêtement fluoré a une épaisseur dans la plage d'environ 1 à 200 nm.

9. Procédé selon la revendication 8, dans lequel l'épaisseur est dans la plage d'environ 10 à 100 nm.

10. Procédé selon l'une quelconque des revendications précédentes, dans lequel le revêtement fluoré est appliqué sur une ou plusieurs surfaces internes de la boîte.

11. Procédé selon l'une quelconque des revendications 1 à 10, dans lequel le revêtement fluoré est appliqué sur une ou plusieurs surfaces internes de la vanne.

12. Procédé selon la revendication 11, dans lequel le revêtement fluoré est appliqué sur une ou plusieurs surfaces internes d'une chambre de mesure de la vanne.

13. Procédé selon la revendication 12, dans lequel le revêtement fluoré est appliqué sur une tige de manoeuvre de la vanne.

14. Procédé selon la revendication 11, dans lequel le revêtement fluoré est appliqué sur une ou plusieurs parties composantes de la vanne choisies dans le groupe constitué d'un joint de tige supérieur, d'un joint de tige inférieur, d'un joint d'étanchéité à lèvre, d'un ressort, d'un corps et d'une bague.

15. Procédé selon l'une quelconque des revendications précédentes, dans lequel le revêtement fluoré est préparé à partir de la copolymérisation plasma de CH₂FCF₃ et d'un ou plusieurs monomères non fluorés supplémentaires.

16. Procédé selon la revendication 15, dans lequel le ou plusieurs monomères non fluorés supplémentaires sont choisis dans le groupe constitué de CH₄, C₂H₆, C₂H₄, N₂, O₂, H₂ C₃COO(C₆H₆)COOCH₃, HO(CH₂)₂OH, C₃H₃N et C₄H₆.

17. Procédé selon l'une quelconque des revendications précédentes dans lequel le revêtement fluoré est appliqué par un processus comprenant les étapes consistant à (i) placer le composant à revêtir dans une chambre, (ii) évacuer la chambre, (iii) amener le gaz CH₂FCF₃ dans la chambre, (iv) appliquer une puissance suffisante pour générer un plasma, (v) allumer le plasma, (vi) éteindre tout plasma qui n'a pas réagi et (vii) rincer la chambre.

18. Procédé selon la revendication 17, dans lequel un ou plusieurs gaz de monomères non fluorés supplémentaires sont amenés dans la chambre.

19. Procédé selon la revendication 18, dans lequel le rapport du débit de gaz CH₂FCF₃ au débit de gaz non fluoré varie continuellement au cours du processus.

20. Procédé selon l'une quelconque des revendications 18 à 19, dans lequel le rapport du débit de gaz de CH₂FCF₃ au débit de gaz non fluoré augmente au cours du processus.

21. Procédé selon l'une quelconque des revendications 18 à 20, dans lequel le gaz est un monomère non fluoré pur au début du processus et un gaz de CH₂FCF₃ pur à la fin du processus.

22. Procédé selon l'une quelconque des revendications 17 à 21, dans lequel le processus est réalisé à une puissance de 50W à 450W.

23. Procédé selon l'une quelconque des revendications 17 à 22, dans lequel le processus est réalisé à une pression gazeuse inférieure ou égale à 70 mTorr.

24. Procédé selon l'une quelconque des revendications 17 à 23, dans lequel le processus est réalisé à un débit de gaz de 50 cm³/min à 200 cm³/min.

25. Procédé selon l'une quelconque des revendications 17 à 24, dans lequel le processus est réalisé à une vitesse de tambour de 1 à 15 tr/min.

26. Procédé selon l'une quelconque des revendications 17 à 25, dans lequel le processus est réalisé à une température de 20°C à 100°C.

27. Procédé selon l'une quelconque des revendications 17 à 26, dans lequel le processus de polymérisation plasma est réalisé à une radiofréquence dans la plage de 2 MHz à 200 MHz.

28. Procédé selon la revendication 27, dans lequel la radio fréquence est d'approximativement 13,56 MHz.

29. Procédé selon l'une quelconque des revendications 17 à 28, dans lequel le plasma est maintenu pendant une durée de 30 minutes, ou sensiblement 30 minutes.

30. Procédé selon l'une quelconque des revendications 17 à 29, dans lequel ledit processus comprend une étape de prétraitement pour retirer la contamination de surface et/ou activer la surface.

31. Procédé selon la revendication 30, dans lequel ladite étape de prétraitement comprend un traitement par plasma des composants avec de l'oxygène ou de l'argon.
